

## UNITED STATES PATENT OFFICE

1,976,544

METHOD OF TREATING MINERAL  
LUBRICATING OILSSterling H. Diggs and James M. Page, Jr., Casper,  
Wyo., assignors to Standard Oil Company, Chi-  
cago, Ill., a corporation of IndianaNo Drawing. Application May 6, 1932,  
Serial No. 609,776

5 Claims. (Cl. 196—13)

This invention relates to a method of treating mineral lubricating oils and it pertains more particularly to the art of preparing lubricating oils stable to oxidation and sludging.

5 Petroleum is essentially a mixture of hydrocarbons comprising several groups or homologous series of compounds, such as the paraffins, hydroaromatics, aromatics, polymethylenes, and various other series of compounds in which the 10 hydrogen to carbon ratio is even lower than in the above classes. A large number of individual compounds of each series are present and have different boiling points, physical and chemical properties. In the various types of crude petroleum 15 commonly known as paraffin base, naphthene or asphalt base, and mixed base oils, these various series of hydrocarbons are present in different proportions. For example, in paraffin base oils such as those from the Appalachian field, there 20 is a relatively high proportion of paraffinic hydrocarbons having a chain structure and a high hydrogen to carbon ratio, whereas in the Gulf Coastal oils there is a high proportion of naphthenic hydrocarbons and hydrocarbons with ring 25 structures and low hydrogen to carbon ratio. The mixed base oils, such as those from Oklahoma and the Mid-Continent area, are in general intermediate between these two extreme types.

In normal refining of crude petroleum, the 30 fractions of varying distillation ranges which are successively obtained by distillation of the oils partake of the general character of the crude; for example, lubricating oils derived from Appalachian crudes will show paraffinic characteristics, whereas the lubricating oils derived from Gulf Coastal oils show naphthenic characteristics. The distillates from the mixed base crudes, such 35 as those from the Mid-Continent area, will show characteristics common to both the naphthenic 40 and paraffinic oils. An important property of paraffinic lubricating oils is their low viscosity temperature coefficient or rate of change of viscosity with temperature. This property makes them particularly suitable for certain lubrication 45 problems where high temperatures are encountered. At low temperatures also, these oils retain their fluidity better, an important consideration in cold weather operation of automobiles, for example. For this reason it is very 50 desirable to separate the mixed base oil into their paraffinic constituents and non-paraffinic constituents.

The paraffinic characteristics of an oil may be 55 expressed by its viscosity index. The expression "viscosity index", as used herein, refers specifically to the index defined by Dean & Davis in Chemical and Metallurgical Engineering, vol. 36, 1929, page 618. The viscosity index of a lubricating oil is an indication of its composition or type, 60 i. e., whether it is a paraffin base or naphthene

base oil. Paraffin base oils are arbitrarily assigned a viscosity index of 100, naphthene base oils are assigned a viscosity index of 0, and mixed base oils lie between these extremes. For example, if an oil shows a viscosity index of about 65 85 to 90, it is evident that the oil is predominately paraffinic in nature.

One of the common ways of increasing the paraffinic content of a lubricating oil is to treat the oil with fuming sulfuric acid. The oil and 70 acid are mixed and agitated in the proportion of about one to two pounds of fuming acid for each gallon of oil. The mixture is then allowed to settle and the acid layer, comprising sulfuric acid and acid sludge, settles to the bottom and is 75 drawn off. The top layer comprises an oil which is high in paraffinic compounds. Also, lubricating oil refined in this way contains a relatively large quantity of sulfonic compounds which must be removed before the oil can be satisfactorily 80 used for most lubricating purposes, and this operation is often expensive and wasteful because of troublesome emulsions which are encountered. The quality of the acid treated lubricating oil can be fairly judged from two of its properties, 85 that is, the viscosity index and stability against sludge formation. The sludge stability is determined by bubbling air at the rate of 10 litres per hour into a 250 cc. sample of oil at 340° F. Samples of 10 grams each are withdrawn at intervals 90 and tested to determine the amount of sludge formed for each 10 grams of oil. When the amount of sludge has increased to 10 mg. the number of hours of oxidation is noted and the sludge stability of the oil is then expressed in 95 hours for 10 mg. of sludge. The amount of sludge is determined by diluting the 10 gram sample of oil with hexane and then filtering off the hexane insoluble residue.

The following table shows the sludge stability 100 of a Mid-Continent lubricating oil distillate of 21.3 A. P. I. gravity, 101.9 Saybolt viscosity at 210° F., and a viscosity index of 54, when treated with different quantities of fuming sulfuric acid.

Table I

| Example | Amt. of fuming acid in pounds | Percent yield | Stability in hours 10 mg. | Viscosity index | 105 |
|---------|-------------------------------|---------------|---------------------------|-----------------|-----|
| 1-----  | 1.5                           | 47            | 66                        | 81              |     |
| 2-----  | 2.7                           | 35            | 125                       | 92              |     |

From the above table it will be observed that a 115 2.7 pound acid treat increased the viscosity index of the oil from 54 to 92, and the treated oil had a sludge stability of 125 hours. Also, it will be noted that the yield is only 35%. From the above data it is apparent that a large quantity of oil is 120

lost when highly stable oils are prepared by acid treating.

Mixed base oils can be made more paraffinic, as indicated by the viscosity index, by extract-

- 6 the naphthenic and naphthenic-like com-  
pounds, or sludge forming hydrocarbons, from  
the oil with organic solvents. The solvent ex-  
traction may be performed with single solvents  
or with mixed solvents, and the extraction may  
10 be performed in one or several stages. Oils pre-  
pared by solvent extraction have very high vis-  
cosity indices, but the oils produced in this way  
are not stable against sludge formation. We have  
15 found that a light sulfuric acid treatment, fol-  
lowing the step of solvent extraction will make the  
oils very resistant to oxidation. We have found  
that the oils prepared by organic solvent extrac-  
tion are particularly unstable as to sludge forma-  
20 tion, but a light acid treatment is also capable  
of making these oils very resistant to sludge  
formation.

We will describe our preferred process by ex-  
tracting a Mid-Continent lubricating oil distillate  
25 with a single organic solvent, di(2 chlorethyl) ether, and then follow this extraction with a light  
sulfuric acid treatment. We will use the same  
oil as described in connection with Table I, that  
30 is, a Mid-Continent lubricating oil distillate of  
21.3 A. P. I. gravity, 101.9 seconds Saybolt vis-  
cosity at 210° F., and a viscosity index of 54. It  
should be understood that our process is applica-  
35 ble to any mixed base lubricating oil. The lubri-  
cating oil and di(2 chlorethyl) ether are mixed in  
the ratio of 3 volumes of solvent for each volume  
of oil, and the mixture is then agitated and heat-  
40 ed to the miscibility temperature. Generally the  
solvent or solvents are miscible with the oil within  
the range of 95-210° F. In this particular exam-  
ple we used a miscibility temperature of 155° F.  
45 After the oil and solvent have been heated to  
the miscibility temperature, the mixture is cooled  
to a temperature below the miscibility tempera-  
ture where the solvent and extract separate from  
50 the highly paraffinic oil. The temperature at  
which this separation is effected is called the "ex-  
traction temperature." In this particular exam-  
ple we used an extraction temperature of about  
55 65° F. It should be understood that the extrac-  
tion temperature may vary with different oils  
and solvents, but generally the extraction tem-  
perature is at least 40° F. below the miscibility  
55 temperature. The uppermost layer of oil com-  
prises the highly paraffinic oil, and this layer is  
referred to as the "raffinate."

55 The solvent and extract are withdrawn from  
the bottom of the agitator, and then the raffinate  
is stripped with an inert gas. Generally, the strip-  
ping is performed at a somewhat elevated tem-  
perature.

60 The raffinate is then given a light sulfuric acid  
treatment. In this example, we used one-half  
pound of 93% sulfuric acid for each gallon of  
raffinate. The oil and acid were mixed and agi-  
tated at about 100° F. for a short time, the acid  
65 layer was allowed to settle and was then drawn  
off. The acid treating may be performed at any  
suitable temperature, but generally a tempera-  
ture within the range of 20 to 200° F. is satis-  
factory. Also, the quantity of acid may be varied  
70 in accordance with the quality of the oil desired,  
but generally from one-fourth to one pound of  
80-98% sulfuric acid will give a very stable oil.  
It should be understood that the more highly  
75 concentrated acid may be used in smaller quan-  
tities.

Typical results illustrating the cooperation be-  
tween solvent extraction and acid treating are  
given in the following table.

Example 1 shows the viscosity index, sludge sta-  
bility and yield of the oil after solvent extraction,  
80 and Example 2 shows the viscosity index, sludge  
stability and yield of the oil after solvent ex-  
traction followed with a light acid treatment.

Table II

85

| Example | Three volumes of di(2 chlorethyl)ether for each gallon of oil |         |       |                           |                 | 90 |
|---------|---------------------------------------------------------------|---------|-------|---------------------------|-----------------|----|
|         | Pounds of sulfuric acid per gallon of ext. oil                | Acidity | Yield | Stability in hours 10 mg. | Viscosity index |    |
| 1.....  | 0                                                             |         |       | 66                        | 93              | 95 |
| 2.....  | 0.5                                                           | 93%     | 55%   | 125                       | 94              |    |

It will be observed from Example 1 in the above  
table that solvent extraction, per se, produced  
an oil of high viscosity index. Before extract-  
ing, the oil had a viscosity index of 54, but by sol-  
vent extraction this was raised to a viscosity index  
of 93. Notwithstanding the high viscosity index,  
the sludge stability of the oil is relatively low.  
By comparing the oil prepared by solvent extrac-  
tion, as set forth in Example 1 of Table II, with  
the oil prepared by acid treatment, as set forth  
in Example 1 of Table I, it will be observed that  
both oils have the same sludge stability, but the  
oil prepared by solvent extraction has a much  
higher viscosity index, that is, the solvent ex-  
tracted oil is more paraffinic than the acid treat-  
ed oil. It will be observed from Example 2 of  
Table II, that a one-half pound 93% acid treat-  
105 applied to the oil in Example 1 of Table II raises  
the sludge stability from 66 hours to 125 hours for  
10 mg. of sludge. Also, the yield of oil is 55%,  
whereas with acid treating per se, see Example 2,  
Table I, the yield is 35% for a 125 hour oil. So,  
by using a light acid treatment after solvent ex-  
traction we can obtain a 55% yield of 125 hour  
110 oil having a viscosity index of 94, whereas by acid  
treating alone, as shown in Example 2 of Table  
I, a 35% yield of 125 hour oil having a viscosity  
index of 92 was obtained. Also, the combination  
115 of solvent extraction and 93% acid treating gave  
an oil with properties that could not be obtained  
with 93% acid treating alone.

A lubricating oil distillate of 22.8 A. P. I. gravity  
and 101 sec. Saybolt viscosity at 210° F. was given  
120 three successive di(2 chlorethyl) ether extrac-  
tions and the raffinate was then given a light  
acid treatment. The volume of chlorinated ether  
used for each extraction was 66% of the volume  
of oil. The following table shows the results from  
125 this treatment.

Table III

130

|                                                                                                                               | Yield vol. | Viscosity 210° F. | Viscosity index | Stability in hrs. 10 mg. | 140 |
|-------------------------------------------------------------------------------------------------------------------------------|------------|-------------------|-----------------|--------------------------|-----|
| Three-stage extraction with di(2 chlorethyl)ether<br>Treatment with 3% of 93% $H_2SO_4$ after the three-stage extraction..... | 60%        | 80.5              | 86.5            | 60                       |     |
|                                                                                                                               | 55%        | 78.6              | 88              | 231                      | 143 |

It will be observed that the light acid treatment  
raised the sludge stability of the solvent extracted  
150

- oil from about 60 hours to 231 hours. Also, the yield of finished product was 55% whereas if fuming acid treatment alone had been used to produce a 231 hour oil, the yield would have been much 5 below 35%.
- It is difficult to explain why such a small amount of acid treatment following solvent extraction of an oil should be so effective in raising the sludge stability of the oil, and at the same time give a 10 high yield of finished product. Possibly the solvents remove the naphthenic compounds that usually protect the sludge-forming compounds, thereby making the sludge-forming compounds of the oil more vulnerable to the action of acids.
- 15 As pointed out above in connection with acid treated oils, a large quantity of soluble sulfonic compounds remained dissolved in the acid treated oil, and it is necessary to remove these sulfonic compounds before the oil can be used for most 20 lubricating purposes. Several processes have been used to remove the sulfonic compounds, the most common of which is to treat the oil with a soap solution. By using our process of solvent extraction followed with a light acid treatment, 25 we overcome the difficulty of having sulfonic compounds dissolved in the raffinate. The solvents remove, among other substances, those compounds which react with sulfuric acid and form sulfonic acids; consequently, when the oil is given a light 30 acid treatment, the soluble sulfonic compounds are not formed to any appreciable extent and their removal constitutes no problem nor entails serious loss of oil.

As pointed out in the above process of chlorinated ether extraction, it is necessary to strip the raffinate of the solvent dissolved therein, but it is very difficult to remove the last trace of solvent from the oil. If all of the halogenated compound is not removed, it will eventually decompose and 35 produce chlorine compounds which are very corrosive. Also, if the oil is extracted with other organic compounds they will dissolve in the raffinate and it is frequently very difficult or even impossible to remove the last trace. Frequently, the 40 color of the oil is impaired when the oil is subjected to severe stripping. Also, if every trace of solvent is not removed from the oil, the oil frequently becomes discolored and deteriorated in other ways. This is particularly true of solvents 45 such as furfural. We have found that by giving the oil a light acid treatment subsequent to the steps of solvent extraction and light stripping, the last traces of solvent that remain in the oil 50 can be very satisfactorily removed and we thereby prevent corrosive and color forming compounds 55 from remaining in the finished oil.

The raffinate, or highly paraffinic oil, which is to be given a light acid treatment, may be obtained by extracting oil with any suitable selective 60 solvent or mixture of solvents which will remove the constituents responsible for low viscosity index. Examples of some of the single solvents suitable for extracting oils are halogenated ethers, nitroaryl compounds, aryl amines, phenols, halogenated esters, and heterocyclic compounds. The 65 following table gives examples of some of the above compounds which may be used for extraction.

Table IV

|    |                                                     |  |
|----|-----------------------------------------------------|--|
| 73 | Methyl 2-chlorethyl ether<br>di(2-chlorethyl) ether |  |
|    | Methyl chloropropyl ether                           |  |
|    | Methyl 2-3 dichloropropyl ether                     |  |
|    | Ethyl 2-3 dichloropropyl ether                      |  |
| 75 | Ethyl chloropropyl ether                            |  |

Table IV—Continued

|                           |    |
|---------------------------|----|
| 2-chlorethyl propyl ether |    |
| Dichlorisopropyl ether    |    |
| Dichlorpropyl ether       | 80 |
| Nitrobenzene              |    |
| Nitrotoluene              |    |
| Nitroxylene               |    |
| Aniline                   |    |
| Phenol                    |    |
| Cresols                   | 85 |
| Cresylic acid             |    |
| Ethyl chloracetate        |    |
| Ethyl dichloracetate      |    |
| Ethyl chloropropionate    |    |
| 2-chlorethyl acetate      | 90 |
| Methyl chloracetate       |    |
| 2-chlorethyl propionate   |    |
| Furfural                  |    |
| Dioxane                   |    |
| Pyridine                  | 95 |
| Nitronaphthalene          |    |
| alpha dichlorohydriins    |    |
| chlorohydriins            |    |

Mixed solvents are also very effective for extracting mixed base lubricating oils, particularly the low boiling ketones, esters or ethers may be mixed with any of the solvents selected from the above Table IV. The following table gives examples of some of the mixed solvents that may be used for solvent extraction.

Table V

|                                                 |     |
|-------------------------------------------------|-----|
| Acetone and nitrobenzene                        |     |
| Acetone and di(2-chlorethyl) ether              | 110 |
| Acetone and furfural                            |     |
| Acetone and dioxane                             |     |
| Acetone and paraldehyde                         |     |
| Acetone and dichlorobenzene                     |     |
| Acetone and ethylene dichloride                 | 115 |
| Acetone and phenol                              |     |
| Acetone and aniline                             |     |
| Acetone and pyridine                            |     |
| Acetone and cresol                              |     |
| Diacetone alcohol and nitrobenzene              | 120 |
| Diacetone alcohol and di(2-chlorethyl) ether    |     |
| Methyl ethyl ketone and di(2-chlorethyl) ether  |     |
| Methyl ethyl ketone and pyridine                |     |
| Methyl ethyl ketone and di(2-chlorethyl) ether  |     |
| Methyl ethyl ketone and phenol                  | 125 |
| Methyl propyl ketone and nitrobenzene           |     |
| Methyl propyl ketone and di(2-chlorethyl) ether |     |
| Methyl isopropyl ketone and furfural            |     |
| Ethyl acetate and nitrobenzene                  |     |
| Ethyl acetate and di(2-chlorethyl) ether        | 130 |
| Ethyl acetate and furfural                      |     |
| Ethyl acetate and nitrotoluene                  |     |
| Ethyl acetate and paraldehyde                   |     |
| Ethyl acetate and phenol                        |     |
| Glycerine and phenol                            | 135 |
| Glycerine and furfural                          |     |
| Glycerine and aniline                           |     |
| Glycol and aniline                              |     |
| Glycol and phenol                               |     |
| Glycol and furfural                             |     |
| Propyl ether and nitrobenzene                   | 140 |
| Isopropylether and nitrobenzene                 |     |
| Isopropylether and chlorinated ethers           |     |
| Ethyl acetate and dioxane                       |     |
| Ethyl acetate and ethylenedichloride            | 145 |
| Methyl acetate and nitrobenzene                 |     |
| Methyl acetate and di(2-chlorethyl) ether       |     |
| Methyl acetate and phenol                       |     |
| Propyl acetate and nitrobenzene                 |     |
| Propyl acetate and di(2-chlorethyl) ether       | 150 |

Table V—Continued

|                                                                                                                                                                                                                                                             |  |
|-------------------------------------------------------------------------------------------------------------------------------------------------------------------------------------------------------------------------------------------------------------|--|
| Propyl acetate and phenol                                                                                                                                                                                                                                   |  |
| Propyl acetate and furfural                                                                                                                                                                                                                                 |  |
| Propyl acetate and dichlorobenzene                                                                                                                                                                                                                          |  |
| 5 Butyl acetate and phenol                                                                                                                                                                                                                                  |  |
| Butyl acetate and furfural                                                                                                                                                                                                                                  |  |
| Butyl acetate and paraldehyde                                                                                                                                                                                                                               |  |
| Butyl acetate and di(2-chlorethyl) ether                                                                                                                                                                                                                    |  |
| Butyl acetate and nitrobenzene                                                                                                                                                                                                                              |  |
| 10 Ethyl propionate and nitrobenzene                                                                                                                                                                                                                        |  |
| Ethyl propionate and di(2-chlorethyl) ether                                                                                                                                                                                                                 |  |
| Ethyl propionate and phenol                                                                                                                                                                                                                                 |  |
| Methyl propionate and nitrobenzene                                                                                                                                                                                                                          |  |
| When any of the solvents set forth in Table IV                                                                                                                                                                                                              |  |
| 15 or V are used to extract mixed base mineral oils, the ratio of solvent to oil is preferably from one to 5 volumes of solvent for each volume of oil. The mixed solvents usually comprise from one to four volumes of ketone, alcohol, ester or ether for |  |
| 20 each volume of the other solvent. For example, one volume of acetone and about two volumes of nitrobenzene are mixed and used to extract one volume of oil. The process, temperatures used, etc., as set forth in connection with the process            |  |
| 25 of using di(2-chlorethyl) ether as a solvent, may in general be successfully used with the solvents given in Tables IV and V.                                                                                                                            |  |

When a mixed base lubricating oil distillate is extracted with any of the above solvents, the raffinate is highly paraffinic, as shown by its viscosity index, but the oil is not as resistant to sludging as would be expected from its high viscosity index. For example a mixed base lubricating oil distillate of 21.6 A. P. I. gravity, 114.30 seconds Saybolt viscosity and a viscosity index of 56.5 was extracted with different mixed solvents, and the following table shows the effect of such extraction upon the viscosity index yield and sludge stability of the oil. One volume of oil 35 was extracted with the mixed solvents set forth 40 in the examples of the following table.

Table VI

| 45<br>Exam-<br>ple | Components                                 | Percent<br>yield | Tot.<br>vol. of<br>com-<br>po-<br>nents | Ratio of<br>com-<br>po-<br>nents | Viscosity<br>index |
|--------------------|--------------------------------------------|------------------|-----------------------------------------|----------------------------------|--------------------|
| 50                 | 1 Acetone and nitrobenzene.....            | 70               | 1.5                                     | 0.5:1                            | 87.5               |
|                    | 2 do.....                                  | 66               | 3                                       | 1:2                              | 93.0               |
|                    | 3 Acetone and di(2-chlorethyl) ether.....  | 75.6             | 2                                       | 1:1                              | 87.5               |
|                    | 4 Acetone and dioxane.....                 | 76               | 2                                       | 1:1                              | 82.5               |
|                    | 5 Acetone and paraldehyde.....             | 60.8             | 3                                       | 2:1                              | 84                 |
| 55                 | 6 Acetone and di-chlorobenzene.....        | 75               | 2                                       | 1.8:0.2                          | 81                 |
|                    | 7 Acetone and ethylene dichloride.....     | 64.6             | 3                                       | 2:1                              | 84.5               |
|                    | 8 Acetone and phenol.....                  | 70.6             | 1.5                                     | 0.5:1                            | 82                 |
|                    | 9 Ethyl acetate and nitrobenzene.....      | 70               | 1.5                                     | 0.5:1                            | 88                 |
| 60                 | 10 Diacetone alcohol and nitrobenzene..... | 66               | 1.5                                     | 0.5:1                            | 83.5               |

It will be observed from the above table, Example 2, that we can raise a 56.5 viscosity index oil to a 93 viscosity index oil, by extracting one volume of the oil with three volumes of solvent, said solvent comprising one volume of acetone and two volumes of nitrobenzene. It will also be observed that the other mixed solvents have varying degrees of effectiveness upon the viscosity index, but all of the mixed solvents raise the viscosity index from 56.5 to a viscosity index of 81 or above. Notwithstanding the high viscosity index, or paraffinicity of these oils, they are susceptible to sludge formation when used under

oxidizing conditions. Most of the oils prepared by the above extraction will produce 10 mg. of sludge in about sixty hours. Also the yield of oil after the acid treatment will be of the order of 5 to 10% below the yield given in the above table with the solvents alone, but if acid treating alone were used to produce oils with 81 to 93 viscosity index and sludge stability of 95 to 150 hours, the yield of finished oil would be very low, and of the order of 35 to 45%. It is apparent from the above data that a light acid treatment following an organic solvent extraction gives a higher yield of finished product than could be obtained by acid treating alone. Also, the oils prepared by solvent extraction and combined light acid treating have a good color, and clay treating may be eliminated.

The term "naphthenic hydrocarbons" is employed in the specification and claims in a generic sense to include the compounds that have a low viscosity index and rapid sludge forming characteristics, examples of which are the aromatic, aromatic-like, olefines, polymethylenes, nitrogen and sulfur compounds.

The method used for mixed solvent extraction followed with a light acid treatment may be the same as set forth hereinabove with single solvents. Also the oil may be extracted with a single solvent, then extracted with a mixed solvent, and then given a light acid treatment to raise the oxidation stability if desired. Also, if desired, the oils may be given a light acid treatment before the step of solvent extraction.

The theory set forth herein to explain the unexpected results obtained by sulfuric acid treating combined with solvent extraction of lubricating oils is not to be considered as limitations upon the scope of our invention, and though the present invention has been described in connection with the details of specific examples, neither is it intended that such examples shall be regarded as limitations upon the scope of the herein described invention except as set forth in the claims.

We claim:

1. The process for preparing a lubricating oil which is highly resistant to sludge formation from a mineral oil containing naphthenic and paraffinic hydrocarbons, which comprises extracting the oil with a solvent containing a halogenated ether and thereby separating the highly naphthenic compounds from the paraffinic compounds, then treating the highly paraffinic fraction with a small quantity of strong sulfuric acid.

2. The process for preparing a lubricating oil which is highly resistant to sludge formation from a mineral oil containing naphthenic and paraffinic hydrocarbons, which comprises extracting the oil with a solvent containing a halogenated ether and a ketone and thereby separating the naphthenic hydrocarbons from the paraffinic hydrocarbons, and then treating the paraffinic hydrocarbons with a small quantity of strong sulfuric acid.

3. The process for preparing a lubricating oil which is highly resistant to sludge formation from a mineral oil containing naphthenic and paraffinic hydrocarbons, which comprises extracting the oil with a mixture of acetone and di(2-chlorethyl) ether and thereby removing the naphthenic hydrocarbons from the paraffinic hydrocarbons, and then treating the highly paraffinic hydrocarbons with a small quantity of sulfuric acid.

4. The process for preparing a lubricating oil which is highly resistant to sludge formation from

90

95

105

110

115

120

125

130

145

5 a mineral oil containing sludge forming and paraffinic hydrocarbons, which comprises heating and agitating the oil with a solvent containing acetone and a chlorinated aliphatic ether, cooling the mixture until the oil separates into a highly paraffinic fraction of hydrocarbons and a fraction of sludge forming hydrocarbons, and then treating the highly paraffinic fraction with 80-98% sulfuric acid in the proportion of about one to one-half pounds of acid per gallon of oil.

10 5. The process for preparing a lubricating oil which is highly resistant to sludge formation from

a mineral oil containing sludge-forming and paraffinic hydrocarbons, which comprises heating and agitating the oil with an organic solvent containing acetone and nitrobenzene, cooling the mixture until the oil separates into a highly paraffinic fraction of hydrocarbons and a fraction of sludge-forming hydrocarbons, and then treating the highly paraffinic fraction of oil with 80-98% sulfuric acid in the proportion of about one to one-half pounds of acid per gallon of oil.

80

85

STERLING H. DIGGS.  
JAMES M. PAGE, JR.

15

90

20

95

25

100

30

105

35

110

115

120